# EUROPEAN PATENT SPECIFICATION

(11) **EP 0 618 081 B1**
(45) Date of publication and mention of the grant of the patent: **15.05.1996**
(21) Application number: 94105080.9
(22) Date of filing: 30.03.1994
(51) Int. Cl.: B41M 5/24, B41M 5/38, B41M 5/035, B41M 5/025

(54) **Thermal transfer image recording method**
Thermisches Übertragungsbildaufzeichnungsverfahren
Méthode pour l'enregistrement d'images par transfert thermique

(30) Priority: 31.03.1993 JP 73972/93
(43) Date of publication of application: 05.10.1994
(73) Proprietor: KONICA CORPORATION, Tokyo 163 (JP)
(72) Inventor: Kawakami, Sota, c/o Konica Corporation, Tokyo (JP); Nakajima, Atsushi, c/o Konica Corporation, Tokyo (JP)
(74) Representative: Henkel, Feiler, Hänzel & Partner

(56) References cited:
- EP-A- 0 489 972

## Description

### Field of the Invention

This invention relates to a thermal-transfer image-recording method capable of providing a recorded image with a high resolving power.

### Background of the Invention

Thermal-transfer recording methods have included, conventionally, a process in which a thermal-transfer recording element comprising a base member provided thereon with a thermally-fusible colorant layer or a colorant layer containing a thermally-sublimable dye is made opposite to an image-receiving element, and a heat source controlled by an electric signal sent from a thermal head or an electricity feeding head is brought into pressure contact from the ink sheet, i.e., the recording element, so that an image can be transferred and then recorded. A thermal-transfer recording has the advantages that noiseless operation, maintenance-free, low cost, easy colored recording and digital recording can be performed, so that thermal recording has been utilized in various fields such as a variety of printers, recorders, facsimiles and the terminals for computers.

In medical and printing fields, on the other hand, there have recently been the demands for a recording process capable of performing the so-called digital recording in which a high resolving powder, a high-speed recording and an image processing can be provided. However, in the thermal-transfer recording processes in which a conventional thermal head or an electricity feeding head has been used as a heat source, an exothermic element has been hardly able to have any high density and any highly resolving image, because of the life of the exothermic element of a head.

For solving the above-mentioned problems, there have been proposed for a thermal-recording technique in which laser beam is used as the heat source, in Japanese Patent Publication Open to Public Inspection (hereinafter referred to as JP OPI Publication) Nos. 49-15437/1974, 49-17743/1974, 57-87399/1982 and 59-143659/1984. In a thermal recording technique in which laser beam is used as the heat source, the resolving power can be enhanced by narrowing the laser spot down. However, when recording an image with a laser beam, the recording time cannot be shortened unless the spots of the recording medium are scanned at a high speed, because it has been usual that the recording is carried out by scanning minute spots. In this case, it is generally disadvantageous to improve a recording speed, as compared to the case where a flood exposure is made or a line thermal head is used. It is also general that a heating given by light is relatively low as compared to a heating given by an exothermic element such as a thermal head. Also from this point, a heat mode recording of the light-heat conversion type utilizing a laser beam or the like is disadvantageous, in the present situation, for improving a recording speed.

On the other hand, JP OPI Publication Nos. 63-35385/1988 and 63-35387/1988 describe each the following technique; a sublimable ink layer and a protective layer containing a thermoplastic resin as a principal component are provided onto a support, and the protective layer is imagewise ablated by laser beam. Thereafter, the surface of the protective layer is brought into close contact with an image-receiving sheet and heat is applied by laser beam or a thermal head from the side of the support having the sublimable ink layer, so that an image information can thermally be transferred thereby to an image-receiving layer. The points of the above-mentioned technique are that a laser beam is output as few as possible, that a protective layer containing a thermoplastic resin as a principal component is fused, and that holes are made by the fused portions pulled to the circumferential portions by the surface tension of the fused thermoplastic resin.

JP OPI Publication No. 4-201486/1992 and EP 489972 (1992) disclose each a technique in which vacuum-evaporated metal layer is applied to a dye-barrier layer, that is equivalent to the aforementioned protective layer.

In these techniques, heating required for an image transfer shall not relatively be limited, because a colorant transfer itself is performed in another means, as compared to a system in which a colorant is transferred by heat applied from the aforementioned laser beam. However, in particular, the above-mentioned patents do not imply any clear cognizance of an exposure light intensity, nor of which layer, an ink layer or a protective layer, can serve as a layer capable of absorbing rays of light.

Furthermore, in the case of using an evaporated metal layer as a protective layer, the metal layer is evaporated on the colorant barrier layer in a vacuum. The evaporation process accompanies a problem that the dye in the colorant layer is sublimated at the time of evaporation.

On the other hand, US Patent Nos. 5,156,938 and 5,171,650 describe each the following technique as another technique; an explosion is produced by irradiating an extremely high power density laser beam to an ink layer or to a layer interposed between a support and an ink layer, and the ink layer is blown off to an image-receiving medium by the explosive force, so that an image can be transferred to the image-receiving element.

### Summary of the Invention

It is an object of the invention to provide an image-recording process and the material for the same, each in which an image having a high resolving power can be recorded and the process can relatively be simplified.

The present inventors have discovered the following technique; a colorant barrier layer is so exploded as to be ablated by irradiating a high power density exposure light such as 100,000 W/cm² or more to the colorant barrier layer, and the colorant can be transferred to an image-receiving layer through the resulting minute holes by applying heat or pressure. The present inventors have also discovered a component effective to the above-mentioned colorant barrier layer, so that the invention could finally be completed. To be more concrete, the above-mentioned objects of the invention can be achieved with the following constitution.

The thermal transfer image recording method of the invention comprises the steps of (1) imagewise exposing a recording element to high intensity light, which comprises a support having thereon a colorant layer containing a colorant, and a colorant barrier layer as defined in claim 1 and containing an infrared absorbing substance and being provided on said colorant layer, to imagewise ablate said colorant barrier layer, (2) contacting the surface of said colorant barrier layer with the surface of image receiving layer of an image receiving element, and (3) transferring colorant of said colorant layer through ablated portion of said colorant barrier layer to said image receiving layer by applying heat or pressure.

Further in the above-mentioned thermal transfer recording process, it can be said to be a preferable embodiment of the invention when the following factors can be satisfied, because the effects of the invention can more be displayed. A high intensity exposure is to have a power density of not lower than 100000 W/cm²; an exposure speed is to be not slower than 1 ms⁻¹; a high intensity exposure is to be made with laser beam; a high intensity exposure is to be made from the side of a colorant barrier layer.

### Brief Description of the Drawings

Fig. 1 is a typical illustration of the time-sequential steps of a recording process in which a thermal-transfer type recording material of the invention; wherein
1 A support for a recording element;
2 A colorant layer;
3 A colorant barrier layer;
4 A support for an image-receiving element; and
5 An image-receiving layer

### Detailed Description of the Invention

As shown in Fig. 1, for example, a thermal transfer recording element of the invention, hereinafter sometimes simply referred to as a recording element, is basically comprised of support 1 laminated thereon with colorant layer 2 and colorant barrier layer 3 in this order.

The supports shall not particularly be limitative, provided that a support is excellent in dimensional stability and durable against a heat source such as laser. The supports applicable thereto include, for example, a thin-leaf paper such as condenser paper and glassine paper; and a heat resistive plastic film such as those made of polyethylene terephthalate, polyamide, polycarbonate, polysulfone, polyvinyl alcohol, cellophane and polystyrene.

The supports are to have a thickness ordinarily within the range of, preferably, 2 to 200µm and, more preferably, 25 to 100µm.

A colorant layer contains a binder besides a colorant. If required, an optional component such as an additive may also be contained therein.

In the invention, it is preferable that a colorant which is to be transferred to an image-receiving layer is to be a thermally diffusible dye. However, without limitation thereto, a colorant may also be other dyes or pigments, and when they may be transferred, it is further allowed to take the so-called thermally fusible transfer system in which a colorant and the binder component thereof may be transferred together.

There is no special limitation to the thermally diffusible dyes, provided that they are thermally diffusible or sublimable. The thermally diffusible cyan dyes include, for example, those of the naphthoquinone type, anthraquinone type and azomethine type, which are described in JP OPI Publication Nos. 59-78895/1984, 59-227948/1984, 60-24966/1985, 60-53563/1985, 60-130735/1985, 60-131292/1985, 61-19936/1986, 61-22993/1986, 61-31292/1986, 61-31467/1986, 61-35994/1986, 61-49893/1986, 61-148269/1986, 62-191191/1987, 63-91287/1988, 63-91288/1988 and 63-290793/1988.

The thermally diffusible magenta dyes include, for example, those of the anthraquinone type, the azo type and azomethine type, which are described in JP OPI Publication Nos. 59-78896/1984, 60-30392/1985, 60-30394/1985, 60-253595/1985, 61-262190/1986, 63-5992/1988, 63-205288/1988, 64-159/1989 and 64-63194/1989.

The thermally diffusible yellow dyes include, for example, those of the methine type, the azo type, the quinophthalone type and the anthraisothiazole type, which are described in JP OPI Publication Nos. 59-78896/1984, 60-27594/1985, 60-31560/1985, 60-53565/1985, 61-12394/1986 and 63-122594/1988.

As for a thermally diffusible dye, it is suitable to make use of an azomethine dye obtained upon making coupling reaction of a compound having an opened- or closed-chain type active methylene group with an oxidant of a p-phenylene diamine or p-aminophenol derivative, and an indoaniline dye obtained upon making reaction of a phenol or naphthol derivative with an oxidation product of a p-phenylene diamine or a p-aminophenol derivative.

Among these dyes, those each capable of forming a chelate compound with a metal ion are preferable.

The dye capable of forming a chelate compound means a dye changeable into a chelate compound after chelating reaction with a metal ion, in more detail, a dye having at least two or more ligands, or a group capable of forming a chelating bond with a metal ion, in the molecule thereof and made these ligand present in a position where a cyclic structure such as 4-, 5-, 6- or 7-member ring can be taken after the ligands are each coordinate to a metal ion. The above-mentioned groups each capable of coordinating to a metal ion, i.e., a chelating group or a ligand, include a group having, for example, -OH, -COOH, -NH₂, -NH-, -N=, -CO-, -O-, -NHCO-, -S-, -SO-, -P=, -NO or -N=N-.

The preferable dyes capable of forming a chelating compound are ones represented by the following Formula 1.
In the above formula 1, X₁ is a group of 5 to 7 atoms necessary to complete an aromatic carbon ring or an aromatic heterocyclic ring provided that at least one atom adjacent to the carbon atom bonded to the nitrogen atom of the azo bonding, is a carbon atom having a substituent capable of forming a chelating bond with a metal ion or a nitrogen atom; X₂ is a group of 5 to 7 atoms necessary to complete an aromatic carbon ring or an aromatic heterocyclic ring: and G is a hydrogen atom or a group capable of forming a chelating bond with a metal ion.

The dyes represented by the above formula 1 include those represented by the following formulas 2 through 8.
In formul 2, Z₁ is a group of atoms necessary to form a 5- or 6-member heterocyclic ring together with the two carbon atom of the benzene ring and Q; Q is -O-, -S-. -N= or -N(R)-, in which R is a hydrogen atom or an alkyl group; R₁ and R₂ are each a hydrogen atom or a monovalent group; and u and w are each an integer of 1 to 5.

The following are exemplified dyes represented by formula 2.
In formula 3, L is -CON(R')-, -COO- or -SO₂-, in which R' is an alkyl group or a hydrogen atom; X₃ is a nitrogen-containing heterocyclic ring or an aromatic carbon ring, provided that the atom adjacent to the carbon atom linked to the azo group is a nitrogen atom or a carbon atom having a group capable of forming chelating bond with a metal ion; and R₃ is a hydrogen atom. an aliphatic group or a heterocyclic group.

Exemplified dyes represented by the above formula 3 are as follows:
In formula 4, R₄ is a substituent; n is an integer of 0 to 3, the plurality of R₄s may be the same or different when n is 2 or 3; and R₅ is a hydroxyl group or an amino group.

Exemplified dyes represented by Formula 4 are as follows:
In formula 5, R₆ and R₇ are each a substituent of the benzene ring and the isoquinoline ring, respectively; p and q are each an integer of 0 to 4, when p and q are each 2 or more, the plurality of R₆s and R₇s may be each the same or different and may link to form a ring, respectively; R₈ is a hydrogen atom, a halogen atom or a monovalent substituent; and G is a group capable of forming chelating bond with a metal ion.

Exemplified dyes represented by Formula 5 are as follows:
In formula 6, R₉ is an alkyl group or a cycloalkyl group; X₄ is a group of atoms necessary to form a 5- or 6-member nitrogen-containing heterocyclic ring together with the carbon atom linked with the azo group and the nitrogen atom linked with said carbon atoms; the heterocyclic ring may have a substituent which may form a 9- or 10-member condensed ring.

Exemplified dyes represented by Formula 6 are as follows:
In formula 7 R₁₀ and R₁₁ is a hydrogen atom or a substituent; X₅ is a group of atoms, necessary to form a 6-member nitrogen-containing heterocyclic ring together with the carbon atom linked with the azo group and the carbon group linked with the hydroxyl group; the heterocyclic ring may have a substituent which may form a condensed ring.

Exemplified dyes represented by Formula 7 are as follows:
In formula 8, R₁₂ is an alkyl group; and R₁₃ is a hydrogen atom or a substituent.

Exemplified dyes represented by Formula 8 are as follows:

| | R₁₂ | R₁₃ | | R₁₂ | R₁₃ |
|---|---|---|---|---|---|
| 8-1 | n-C₅H₁₁ | 3-CH₃ | 8-2 | n-C₃H₇ | 3-CH₃ |
| 8-3 | n-C₆H₁₃ | 3-CH₃ | 8-4 | n-C₄H₉ | 3-CH₃ |
| 8-5 | i-C₃H₇ | 3-CH₃ | 8-6 | CH₂CH(C₂H₅)C₄H₉ | 3-CH₃ |
| 8-7 | n-C₅H₁₁ | H | 8-8 | C₂H₄OC₂H₅ | 3-CH₃ |
| 8-9 | CF₂CF₃ | 3-CH₃ | 8-10 | n-C₄H₉ | 2-F |
| 8-11 | n-C₄H₉ | 3-OCH₃ | 8-12 | CF₃ | 3-C₂H₅ |

Other than the above dyes, the following thermally diffusible dyes, for example, can be use in the invention.
The thermally diffusible dyes may be used in an amount within the range of, ordinarily, 0.1 to 20 g per m² of the support used and, preferably, 0.2 to 5 g per m². In the colorant layer, the thermally diffusible dye content is within the range of, ordinarily, 5 to 70% by weight and, preferably, 30 to 70% by weight.

As for the binders applicable to a colorant layer, any resins known in the thermal-transfer recording field may be used. For this purpose, the following polyvinyl acetal type resins and cellulose type resins may preferably be used, provided, however, that the binders of the invention shall not be limited thereto.

The polyvinyl acetal type resins include various kinds of compounds according to the acetalized degrees and the contents of an acetyl group, and a residual group such as hydroxyl group. The typical examples thereof may include polyvinyl acetoacetal, polyvinyl butyral.

The cellulose type resins include, for example, nitrocellulose, ethyl cellulose, hydroxyethyl cellulose, ethylhydroxyethyl cellulose, hydroxypropyl cellulose, methyl cellulose, cellulose acetate and cellulose butyrate. Among them, nitrocellulose is particularly preferable.

Besides the above, the other resins may be used which are known in the thermal-transfer recording field include, for example, acrylic resin, methacrylic resin, polycarbonate, polyvinyl alcohol, polyvinyl formal, polyvinyl ether, polyvinyl pyrrolidone, polystyrene, a polystyrene copolymer and ionomer resin.

From the above-given binders, one or more kinds of them can suitably be selected to be used. It is preferable to compound the above-mentioned binders in a proportion within the range of, ordinarily, 30 to 70% by weight of the whole colorant layer. In a colorant layer, the weight ratio of the binder thereof to the thermally diffusible dye thereof is to be within the range of, preferably, 1:10 to 10:1 and, particularly, 2:8 to 8:2.

A colorant layer may have any thickness, provided that the colorant layer can be controlled to be peeled off from an image receiving element and that the colorant thereof can be controlled to be transferred by applying heat energy. The thickness of a colorant layer is to be within the range of, ordinarily, 0.2 to 10µm and, preferably, 0.4 to 5µm.

In the invention, an additive to be added to a colorant layer include, for example, fluororesin, a surfactant, wax, higher aliphatic acid, higher aliphatic alcohol, higher aliphatic ether, fine metal powder, silica gel, carbon black, organic filler, inorganic filler, and a hardener reactive with a binder component, such as a radiation-active compound, e.g., isocyanate, acrylic acid and epoxy, as well as modified silicone resin. For the purpose of promoting a transfer, it is further allowed to make use of a thermally fusible substance such as higher aliphatic ester described in, for example, JP OPI Publication No. 59-106997/1984.

The amounts of the additives to be added cannot be determined without distinction, because of the various kinds of additives and the various purposes for adding them. Usually, as the whole of them, it is preferable to add them in a proportion of not more than 50% by weight of a binder used.

The typical examples of the above-mentioned modified silicone resins include polyester-modified silicone resin, acryl-modified silicone resin, urethane-modified silicone resin, cellulose-modified silicone resin, alkyd-modified silicone resin and epoxy-modified silicone resin. They may be used independently or in combination.

The above-mentioned modified silicone resins may be compounded in a proportion within the range of, ordinarily, 0.01 to 10% by weight of a colorant layer and, preferably, 0.01 to 2.0% by weight thereof.

A colorant layer can be formed by the following manner. The foregoing thermally diffusible dye, binder and, if required, an additive are each dissolved or dispersed in a solvent, so that a coating solution can be prepared, and the resulting coating solution is coated over a support and then dried up.

The binders may be used not only by dissolving one or more kinds thereof in a solvent, but also by latex-dispersing them.

The solvents include, for example, water, an alcohol such as ethanol, propanol and butanol, cellosolve, an ester such as ethyl acetate and butyl acetate, an aromatic compound such as toluene, xylene and chlorobenzene, a ketone such as acetone and methyl ethyl ketone, an ether such as tetrahydrofuran and dioxane and a chlorine-containing solvent such as chloroform and trichloroethylene. These solvents may be used independently or in combination.

The coating solution may be coated by a commonly known coating process such as a sequentially coating process in which a gravure-roll is used, an extrusion coating process, a wire-bar coating process and a roll coating process.

A barrier layer is to be provided at least with a property that it cannot be permeated with the colorant or the thermally diffusible dye of a colorant layer even when applying heat or pressure and another property that it can absorb any high intensity exposure light. For providing it with the properties, it is preferable that a colorant barrier layer is to contain a resin, in which (1) a water-soluble resin, (2) a resin having an ion bond, or (3) a resin having a Tg (or a glass-transition point) of not lower than 120°C, preferably not lower than 150°C and, more preferably not lower than 200°C, is contained as the principal component.

The water soluble resin which may be used in the invention is a resin capable of being dissolved in water in a concentration of not less than 1 % by weight, preferably not less than 2 %. The above solubility of the resin is not limited that at an ordinary temperature. Temperature for dissolving the resin can be changed according to necessity. A resin can be used which can be dissolved in water with a concentration of not less than 1 % by weight at a temperature 0 to 100°C.

The water-soluble resins include, for example, gelatin, polyvinyl alcohol, water-soluble polyvinyl formal, water-soluble polyvinyl acetal, water-soluble polyvinyl butyral, polyvinyl pyrrolidone, water-soluble polyester, water-soluble nylon, polyacrylic acid, water-soluble polyurethane, methyl cellulose, hydroxyethylcellulos, hydroxypropyl cellulose, and carboxyl cellulose. It is also allowed to use the copolymers of the monomer components constituting the above-given resins. At the time of preparation of coating solution, it is preferable to dissolve gelatin at a temperature of not lower than 40°C and to dissolve methyl cellulose at a temperature of not higher than 10°C.

The term, a resin having a ion-bond, means a resin having an ion-bonded group that is, an acidic or basic group, in the principal or side chain of a macromolecule.

The acidic groups include, for example, -COO⁻, -SO₃⁻ and -PO₃⁻. The basic groups include, for example, -NH₂,
and -N=.

The resins each having an ion-bond include, for example, those having both of an acidic group and a basic group, and those each having an acidic group, containing a divalent metal ion and having a cross-linking structure through the metal ion. It is preferred that a resin having an ion bond, that is related to the invention, has at least one or more of the ion-bonded groups per 100 repetition monomer units. However, a resin not always having such a repetition monomer unit as mentioned above can also suitably be used.

The resins having an ion bond include, for example, a resin containing styrene substituted with a sulfo group, acrylic acid, methacrylic acid, phthalic anhydride, or the like, each added with Na⁺, K⁺, Ca²⁺, NH⁺ or the like as a counter ion, besides an ionomer resin and so forth. Further, gelatin and casein may also be used preferably.

The resins each having a Tg of not lower than 120°C include, for example, polyvinyl chloride, polystyrene, polyaryl methacrylate, polybenzyl methacrylate, polycarbonate, nylon, polyphenylene oxide, polyphenylene sulfide, gelatin and polyparabanic acid. A resin having a Tg of not lower than 120°C is also preferably used, that is, a copolymer of a monomer component of styrene, vinyl chloride, methyl methacrylate, aryl methacrylate, acrylonitrile, ethylene oxide, benzyl methacrylate or cyclohexyl methacrylate. It is further preferable to use a thermosetting resin without having any glass transition point.

Among these resins usable for the colorant barrier layer, water-soluble ones are preferable. As the water-soluble resin, gelatin, polyvinylpyrrolidone, methylcellulose, hydroxyethylcellulose, hydroxypropyl-cellulose, carboxylcellulose are particularly preferable. These water-soluble resins are well mixed with the water-soluble infrared absorbing dyes after-mentioned.

The proportion of a resin component to a colorant barrier layer is preferably within the range of 50 to 99% by weight of a colorant barrier layer. Among the resin components, the proportion of the foregoing resin component (1), (2) or (3) of to the whole resin component is preferably not less than 50% by weight, more preferably not less than 70% by weight and, most preferably not less than 90% by weight based on the total weight of the barrier layer.

The colorant barrier layer contains an infrared absorbabing substance for absorbing a high intensity exposure light and converting the absorbed light to heat. The infrared absorbing substances are preferably ones which absorb infrared radiation having a wavelength of not shorter than 650 nm.

As for the infrared absorbing dyes, any one of them can be used, provided that they can absorb infrared rays of not lower than 700nm. However, for effectively achieving the invention, it is preferable to make use of a dye having a molar extinction coefficient of not less than 50,000 and, preferably, not less than 100,000, in a wavelength showing the strongest absorption within the range of 700nm to 1200nm.

An infrared absorbing dye applicable to the invention preferably has good compatibility with the binder for the colorant barrier layer of the invention. An infrared absorbabling dye of the invention also preferably dissolves, in a proportion of not less than 0.1% and, particularly, not less than 1%, in at least water or an organic solvent, provided that there shall not exclude those capable of being mixed with a binder for a colorant barrier layer, by dispersing them in at least water or an organic solvent.

It is further preferable that an infrared absorbing dye for use in the invention could have the another characteristic that it can readily be decomposed by irradiating heat from a laser beam. For example, when raising room temperature at a rate of 10°C/minute under nitrogen flow, it is preferred that a temperature showing a 10% weight reduction is at least not higher than 500°C, preferably not higher than 400°C and, more preferably not higher than 350°C. However, the above-mentioned heat decomposable characteristics shall not be indispensable to the invention.

It is allowed to use such an infrared absorbing dye as given in JP Application No. 4-334584/1992, p.7, and carbon black. For example, it is allowed to use the following dyes selected from the near infrared absorbing dyes given in "Kinou Zairyo" (Functional Materials), June, 1990 Issue, pp. 64-68, the functional dyes for optical recording use given in "Shikizai" (Colorant), Vol. 61 (1988), pp. 218-223; the cyanine dyes, Squarylium dyes, azulenium dyes, phthalocyanine type, naphthalocyanine dyes, anthraquinone dyes, dithiol metal complex salt dyes, indoaniline metal complex dyes, intermolecular CT complex dyes, transition metal chelate dyes, and aluminium diimmonium dyes.

Infrared absorbing dyes preferably usable in the invention to convert light to heat are those represented by the following formulas I to XI or XII. Among the infrared absobing dyes represented by formula I to XI or XII, water-soluble ones are preferable. The water-soluble infrared absorbing dyes preferably used in the invention are those each having a acid group such as a sulfo group, a carboxyl group and a phosphono group, in which ones having sulfo group are particularly preferable.
In the above formula I, Z₁ and Z₂ are each independently a group of atoms necessary to form a substituted or unsubstituted pyridine ring, a substituted or unsubstituted quinoline ring or a substituted or unsubstituted benzene ring or a substituted or unsubstituted naphthalene ring, Z₁ and Z₂ may be include =N⁺- or -N(R₆)- bond when they are a pyridine ring or a quinoline ring; Z₃ and Z₄ are each independently a group of atoms necessary to form a substituted or unsubstituted pyridine ring or a substituted or unsubstituted quinoline ring, Z₃ and Z₄ may be include =N⁺- or -N(R₆)- bond; Y₁ and Y₂ are each independently a dialkyl substituted carbon atom, a vinylene group, an oxygen atom, a sulfur atom, a selenium atom or a nitrogen atom linked with a substituted or unsubstituted alkyl group or a substituted or unsubstituted aryl group; R₁ and R₆ are each independently a substituted or unsubstituted alkyl group; R₂, R₄, and R₅ are each independently a hydrogen atom or a substituted or unsubstituted alkyl group, R₂ may link with R₄ to form a ring; R₃ is a hydrogen atom, a halogen atom, a substituted or unsubstituted alkyl group, are each independently a substituted or unsubstituted aryl group or a nitrogen atom linked with an alkyl group or an aryl group; at least one of the groups represented by the above Z₁ through Z₄ and R₁ through R₆ has a sulfo group, a carboxyl group or a phosphono group; X⁻ is an anion; m is 0 or 1 and n is 1 or 2, provided n is 1 when an intramolecule salt is formed. Among the dyes represented by the above formula I, ones having in which at least one of the groups represented by R₁ to R₆ has a sulfo group, a carboxyl group or a phosphono group, particularly a sulfo group, are preferable.
In formula II, Y₃ and Y₄ are the same as Y₁ and Y₂ defined in the above formula I, resprctively; Z₃ and Z₄ are the same as Z₁ and Z₂ defined in formula I, respectively; R₈, R₁₀, R₁₄ and R₁₆ are each independently a substituted or unsubstituted alkyl group, a halogen atom or a hydrogen atom, R₈ and R₁₀, R₁₄ and R₁₆ each may be bonded to form a ring; R₉, R₁₁, R₁₂, R₁₃ and R₁₅ are each independently a substituted or unsubstituted alkyl group, a halogen atom or a hydrogen atom; R₇ and R₁₇ are each independently a substituted or unsubstituted alkyl group or a hydrogen atom; and X⁻, m and n are each the same as X⁻, m and n defined in formula 1, respectively. Among the dyes represented by the above formula, ones in which at least one of the groups represented by R₇ to R₁₇ has a sulfo group, a carboxyl group or a phosphono group are preferable. Ones having a sulfo group is particularly preferable.
In formula III, R₁₈, R₁₉ and R₂₀ are each independently a hydrogen atom, a substituted or unsubstituted alkyl group -N(R₂₃)(R₂₄), =N⁺(R₂₃)(R₂₄) or a sulfo group, in which R₂₃ and R₂₄ are each independently a substituted or unsubstituted alkyl group; Y is a carbon atom or a nitrogen atom; R₂₁ and R₂₂ are each independently a hydrogen atom or a substituted or unsubstituted alkyl group; X⁻ an anion; m is 0 to 5 and n is 1 or 2. Among the dyes represented by formula III, ones in which at least one of the groups represented by R₁₈ to R₂₄ has a sulfo group, a carboxyl group or a phosphono group, particularly a sulfo group, are preferable.
In the above formula IV, R₂₅, R₂₆, R₂₇ and R₂₈ are each independently a hydrogen atom or a substituted or unsubstituted alkyl group. Among the dyes represented by formula IV, ones in which at least one of the groups represented by R₂₅ to R₂₈ has a sulfo group, a carboxyl group or a phosphono group, particularly sulfo group, are preferable.
In the above formula V, R₂₉ and R₃₀ are each independently a substituted or unsubstituted alkyl group; and R₃₁ and R₃₂ are each independently a hydrogen atom or a substituted or unsubstituted alkyl group. Among the dyes of formula V, ones in which at least one of the groups represented by R₂₉ to R₃₀ has a sulfo group, a carboxyl group or a phosphono group, particularly sulfo group, are prefeable. Further, R₃₁ and R₃₂ may be substituted with a sulfo group, a carboxyl group or a phosphono group.
In formula VI, R₃₃, R₃₄ and R₃₅ are each independently a hydrogen atom, a substituted or unsubstituted alkyl group; and X⁻ is an anion. Among the dyes of formul VI, ones in which at least one of the groups represented by R₃₃ to R₃₅ has a sulfo group, a carboxyl group or a phosphono group, particularly sulfo group, are prefeable.
In formula VII, R₃₆ and R₃₇ are each independently a hydrogen atom, a sulfo group, a carboxyl group. a phosphono group or a substituted or unsubstituted alkyl group; and R' and R'' are each independently a hydrogen atom, a substituted or unsubstituted amino group or a substituted or unsubstituted alkyl group. As the substituted alkyl group represented by R₃₆ and R₃₇, those usbstitued with a sulfo group, a carboxyl group or a phosphono group,
In formula VIII, R₃₈ is a hydrogen atom, a substituted or unsubstituted amino group, a substituted or unsubstituted amido group or a substituted or unsubstituted alkyl group; R₃₉ and R₄₀ are each independently a hydrogen atom or a substituted or unsubstituted alkyl group; and R₄₁ is a hydrogen atom, a sulfo group, a carboxyl group, a phosphono group or a substituted or unsubstituted alkyl group, M is an metal atom; and X⁻ is an anion. As the above substituted alkyl group represented by R₃₈ to R₄₁, those substituted with a sulfo group, a carboxyl group or a phosphono group are preferable. As the metal represented by M, Cu and Ni are preferable.
In formula IX, R₄₂ is a hydrogen atom or a substituted or unsubstituted alkyl group; R₄₃ is a a hydrogen atom, an amido group, a nitro group, a sulfo group, a carboxyl group, a phosphono group or a substituted or unsubstituted alkyl group; and R₄₄ is s hydrogen atom, a sulfo group, carboxyl group, a phsphono group or a substituted or unsubstituted alkyl group. As the substituted alkyl group represented by R₄₂ to R₄₄, those substituted with a sulfo group, a carboxyl group or a phosphono group are preferable.
In the above formula X, R₄₄ and R₄₅ are each independently a hydrogen atom a sulfo group, a carboxyl group, a phosphono group or a substituted or unsubstituted alkyl group; R₄₆, R₄₇, R₄₈ and R₄₉ are each independently an alkyl group which may be the same or different; and n is 0 to 4. As the substituted alkyl groups represented by R₄₄ and R₄₅, those substituted with a sulfo group, a carboxyl group or a phosphono group are preferable.
In formula XI, R₅₁ and R₅₂ are each independently a hydrogen atom, a sulfo group, a carboxyl group, a phosphono group or a substituted or unsubstituted alkyl group; M is a divalent or trivalent metal atom; and n is 2 or 3. As the substituted alkyl groups represented by R₅₁ and R₅₂, those substituted with a sulfo group, a carboxyl group or a phosphono group are preferable.
In formula XII. R₅₃, R₅₄, R₅₅ and R₅₆ are each independently a hydrogen atom, a sulfo group, a carboxyl group, a phosphono group or a substituted or unsubstituted alkyl group; and M is a divalent metal atom. Preferable substituents of the alkyl groups reprented by R₅₃ to R₅₆ are each a sulfo group, a carboxyl group or a phosphono group. Among these infrared absorbing dyes, cyanine dyes represented by formulas I or II, anthraquinone dyes represented by formula VII, and chelate dyes represented by formula VIII, X, XI or XII are preferable. Cyanine dyes of formula I or II each having a sulfo group are particularly preferable.

Among these infrared absorbing dyes, cyanine dyes represented by formula I or II, anthraquinone dyes reprented by formula VII, and chelate dyes represented by formula VIII, X, XI or XII are preferable. Cyanine dyes of formula I or II each having a sulfo group are particularly preferable.

The followings are exemplified water-soluble infrared absorbing dye represented by Formula I to XI or XII.
Further, dyes represented by formulas each the same as Formulas I to XII except that which do not have neither sulfo group, carboxyl group nor phosphono group are also may be used.

When the colorant barrier layer comprises a water-insoluble resin, infrared absorbing dyes described in JP O.P.I. Publications 62-12345 (1987) and 3-146565 (1991) can be used.

When the wavelength of the exposure light is in the infrared region, it is preferable that the light-absorbing substance contains the foregoing infrared-absorbing dye in a proportion within the range of 1 to 50% by weight in the colorant barrier layer. If the infrared absorbing substance does not deteriorate the barrier function of the foregoing infrared-absorbing dye of a colorant barrier layer, the near infrared absorbing dye can further be added in a further amount.

Besides the above colorant barrier layer can also contain, if required, additives such as a surfactant for improving coatability, a conductive compound as an antistatic agent, and a releasing agent for preventing blocking and a matting agent.

The layer thickness of a colorant barrier layer is to be as thin as possible, provided that the barrier function cannot be deteriorated. To be more concrete, the thickness thereof is to be within the range of 0.1 to 2.0µm and, preferably, 0.1 to 1.0µm, provided, however, that the layer thickness thereof shall not be limited thereto, because ablation can be made even if the layer thickness is thicker, when an exposure light intensity is satisfactorily high.

If required, a colorant barrier layer may be formed of a plurality of layers by which the functions are separated. The functions to be separated thereby include, for example, colorant barrier property, conductivity, light absorbancy and blocking resistance. These functions may be provided separately to a plurality of layers.

A colorant barrier layer can be coated in the same manner as in the case of the foregoing colorant layer.

In the invention, if required, besides the colorant layer and colorant barrier layer, other layers may be provided. For example, between the support and the colorant layer, a sublayer can be interposed for enhancing adhesion and so forth. An intermediate layer may be provided between the colorant layer and the colorant barrier layer, which has a heat insulating or an adhering effect. And, to the rear side of a support, (that is, the opposite side thereof to a colorant layer), a backing layer may also be provided for the purposes of endowing running stability, heat-resistance, antistaticity. The above-mentioned backing layer preferably has a layer thickness within the range of 0.1 to 1µm.

Further to a recording element, a series of perforations, a detection mark for detecting the positions of every area having different hues, and so forth may be provided, so as to meet the convenience for use.

Now, an image-receiving material applicable together with a recording material of the invention will be detailed below.

An image-receiving element is comprised of a support and an image-receiving layer. However, an image-receiving material may also be formed of an image-receiving layer which is self-supported.

The supports include, for example, those made of the following materials; paper, coated paper, synthetic paper such as those made of polypropylene and polystyrene, and those made of the compounded materials thereof pasted on a paper or a plastic film, those made of a white or transparent polyethylene terephthalate film, those made of a white or transparent polyvinyl chloride sheet, and those made of polyolefin-coated paper. The thicknesses of the supports are to be within the range of, normally, 20 to 300µm and, preferably, 30 to 200µm.

An image-receiving layer is formed of a binder for image-receiving layer and a variety of additives. The binders for image-receiving layer include, for example, a polyvinyl chloride resin, a copolymeric resin of vinyl chloride and other monomer such as alkyl vinyl ether and vinyl acetate, a polyester resin, a poly acrylate, polyvinyl pyrrolidone, polycarbonate, cellulose triacetate, a styrene acrylate resin, a vinyl toluene acrylate resin, a polyurethane resin, a polyamide resin, a urea resin, a polycaprolactone resin, a styrene-maleic anhydride resin and a polyacrylonitrile resin.

The above-given resins may be synthesized afresh. However, those available on the market may also be used. In any case, from the viewpoint of physical properties, a resin having a Tg within the range of -20 to 150°C and, particularly, 30 to 120°C is preferable as a binder for image-receiving layers. Also, a resin having a weight average molecular weight within the range of 2,000 to 100,000 is preferable.

When forming an image-receiving layer, a variety of the above-mentioned resins may also be cross-linked or hardened by utilizing the reaction active sites thereof (provided, when there is no reaction active site, the reaction active sites are endowed) and then by applying radiation, heat, moisture, a catalyst or the like. When this is the case, it is allowed to make use of a radiation active monomer such as epoxy and acryl, and a cross-linking agent such as isocyanate.

It is preferable that the image-receiving layer contains a metal ion-containing compound as a metal source to form a chelate compound with a diffusible dye transferred from a image recording element. As for the metal ion-containing compounds, anyone of organic and inorganic compound each have a metal ion bonded with ion bonding or coordinate bonding thereto. Generally from the view points of a solubility and a handling convenience, a salt or complex of a low-molecular organic compound are preferably used, however, the metal ion-containing compound are limited hereto.

As the above metal, monovalent or polyvalent metal of Groups I to VIII of the Periodic Table can be used. Among them, Al, Co, Cu, Fe, Mg, Mn, Mo, Ni, Sn, Ti and Zn, particularly Cu, Cr, Co and Zn, are preferable. Examples of the metal ion-containing compound suitably used include salts of Ni²⁺, Cu²⁺, Cr²⁺, Co²⁺ or Zn²⁺ with an aliphatic acid such as acetic acid and stearic acid, and salts of these metal ions with an aromatic carboxylic acid such as benzoic acid and salicylic acid.

Further, complexes represented by the following formula C-1 are particularly preferably used.

[M(Q₁)_{ℓ}(Q₂)ₘ(Q₃)ₙ]^{P+}(Y⁻)^{P} (C-1)

wherein M is a metal ion; preferably Ni²⁺, Cu²⁺, Cr²⁺, Co²⁺ or Zn²⁺; Q₁, Q₂ and Q₃ are each independently a ligand compound capable of forming a coordinate bond with a metal ion represented by M, which may be the same or different. The above ligand compound represented by Q₁ to Q₃ may be selected from ligand compounds described in "Chelate Chemistry (5)", p.p. 1-372, Konando 1975. Y⁻ is an anion, preferably an organic anion, such as tetraphenylboron anion and alkylbenzene-sulfonate anion. ℓ is 1, 2 or 3; m is 1, 2 or 0; and n is 1 or 0, and these numbers are defined according to the number of ligand of the compound represented by Q₁, Q₂ and Q₃, or the number of coordinate, 4-coordinate or 6-coordinate, of the complex. P is 0, 1 or 2. When the ligand compound represented by Q is an anionic compound, and cation of metal ion of M is neutralized by anion of compound Q, P is 0. The anionic compounds preferable be used are those represented by the following formula C-2:
wherein R₅₇ and R₅₈ are each a hydrogen atom an alkyl group or an aryl group which may be the same or different; and R₅₉ is a hydrogen atom, an alkyl group, an alkoxyl group, a halogen atom or an alkoxycarbonyl group.

A metal source M²⁺(X⁻)₂ is formed from the above anionic compound (X⁻) of formula C-2 and a metal ion M²⁺. Compounds each having -COOCH₃ or -COOC₂H₅ as the group represented by R₄₆ are preferable. As metal represented by the above M is preferably Ni. The metal ion-containing compound is contained in the image receiving layer in a content of 0 to 80 % by weight. The content can be varied depending on the kind of the metal ion-containing compound and the thickness of the image receiving layer.

The followings are the examples of the anionic compound represented by formula C-2.

To an image-receiving layer, a peeling agent, an antioxidant, a UV absorbent, a light stabilizer, a filler and a pigment may be added. And, a plasticizer, a heat solvent and so forth may also be added to serve as a sensitizer.

A peeling agent is capable of improving a recording material peeling property. For example, they include silicone oil including the so-called silicone resin; a solid wax such as polyethylene wax, alkyd wax and Teflon powder; and a fluorine type or phosphoric acid ester type surfactant. Among them, silicone wax may preferably be used.

The amounts of a simply-adding type silicone oil to be added may not be determined uniformly, because they are so added as to meet the various kinds thereof. However, they may be added in a proportion within the range of 0.5 to 50% by weight and, preferably, 1 to 20% by weight to a binder for an image-receiving layer to be used.

As for a reaction-setting type silicone oil, there include, for example, those prepared by reaction-setting an amino-denatured silicone oil with an epoxy-denatured silicone oil. As for a catalyst-setting type or a light-setting type silicone oil, there include, for example, those of KS-705F-PS, KS-705F-PS-1 and KS-770-PL-3 which are catalyst-setting type silicone oils manufactured by Shinetsu Chemical Industrial Co.; and KS-720 and KS-774-PL-3, which are light-setting type silicone oils manufactured by Shinetsu Chemical Industrial Co..

The above-mentioned light-setting type silicone oils are to be added preferably in a proportion within the range of 0.5 to 30% by weight to a binder for an image-receiving layer to be used.

It is also allowed that the above-mentioned peeling agent is dissolved or dispersed in a suitable solvent, and the resulting solution or dispersion is then coated on a part of the surface of an image-receiving layer and then dried, so that a peeling layer can be provided.

As for the above-mentioned antioxidants, there may include, for example, the compounds given in JP OPI Publication Nos. 59-182785/1984, 60-130735/1985 and 1-127387/1989; and a compound well-known as a compound capable of improving an image durability of photographs or other image-recording elements.

As for the above-mentioned UV absorbents and light stabilizers, there may include, for example, the compounds given in JP OPI Publication Nos. 59-158287/1984, 59-196292/1984, 61-283595/1986, 62-229594/1987, 63-74686/1988, 63-145089/1988, 63-122596/1988 and 1-204788/1989; and the compounds well-known as a compound capable of improving an image-durability of photographs and other image-recording elements.

As for the fillers, there may include, for example, inorganic or organic fine particles. As for the inorganic particles include, for example, those of silica gel, calcium carbonate, titanium oxide, acid clay, active clay or alumina. As for the organic particles include, for example, resin particles such as those of fluororesin, guanamine resin, acrylic resin and silicone resin.

These inorganic or organic fine particles are preferably added in a proportion within the range of 0.1 to 70% by weight, provided, however, that the amounts thereof to be added may be varied according to the specific gravities thereof.

As for the above-mentioned pigments, there may include. for example, those of titanium white, calcium carbonate, zinc oxide, barium sulfate, silica, talc, clay, kaolin, activated clay and acid clay.

As for the above-mentioned plasticizers, there may include, for example, those of a phthalic acid ester, a trimellitic acid ester, a pyromellitic acid ester, an adipic acid ester, other oleic acid esters, a succinic acid ester, a maleic acid ester, a sebacic acid ester, a citric acid ester, epoxidated soybean oil, epoxidated linseed oil, epoxystearic acid, an orthophosphoric acid ester, a phosphorous acid ester and a glycol ester.

The whole additive is to be added in a proportion ordinarily within the range of 0.1 to 50% by weight to a binder for an image-receiving layer used.

An image-receiving layer can be formed in the following process; for example, a coating process in which a coating solution is prepared by dispersing or dissolving the components of the image-receiving layer in a solvent, and the resulting coating solution is coated on the surface of a support and then dried; or a lamination process in which a mixture comprising the components of the image-receiving layer is fused to be extruded, so that the extrusion thereof is laminated on the surface of a support.

As for the solvents applicable to the above-mentioned coating processes, there may include, for example, tetrahydrofuran, methyl ethyl ketone, toluene, xylene, chloroform, dioxane, acetone, cyclohexane and butyl acetate.

When making use of the above-mentioned lamination process, a co-extrusion process may also be used in the case where a support is made of a synthetic resin.

An image-receiving layer may be formed over the whole surface of a support, or may also be formed on a part of the surface of the support.

The thickness of an image-receiving layer is of the order within the range of, generally, 1 to 50µm and, preferably, 2 to 10µm. On the other hand, when a self-supportable image-receiving layer itself forms an image-receiving material, the thickness thereof is of the order within the range of, generally, 60 to 200µm and, preferably, 90 to 150µm.

On the surface of an image-receiving layer, an over-coat layer may also be laminated with the purposes of preventing any fusion, improving an image preservability, and so forth. The over-coat layer may be formed in a gravure-coating process, a wire-bar coating process, a roll coating process, other well-known coating processes, or a lamination process. The thickness of the layer is ordinarily within the range of 0.05 to 3µm.

When an image-receiving element comprises a support and an image-receiving layer, a cushion layer may be interposed between the support and the image-receiving layer, with the purposes of reducing a noise, and transferring and recording an image, with an excellent image-reproducibility, so as to correspond an image information.

The materials for a cushion layer may include, for example, a urethane resin, an acrylic resin, an ethylene type resin, an epoxy resin and a butadiene rubber. The thickness of a cushion layer is preferably within the range of 5 to 25µm.

Now, a thermal transfer-recording process for forming an image of the invention will be detailed below.

As shown in Fig. 1, an image-forming process is comprised of a step in which a colorant barrier layer is ablated imagewise by making a high intensity exposure from the side of a recording element and, preferably, from a colorant barrier layer, and another step in which the ablated recording element and an image-receiving element is so put one upon another as to make the colorant barrier layer and an image-receiving layer face to face, and heat or pressure is then applied to the whole surfaces thereof.

As for the light sources for making a high intensity exposure, there may include, for example, those of Xenon light, halogen light, semiconductive laser beam, He-Ne laser beam, Ar laser beam, YAG laser beam and carbonic acid gas laser beam. From the viewpoint of the handling convenience, semiconductive laser beam is preferably used as the Light source. However, the light sources shall not be limited thereto.

The power density of an exposure is, preferably, not lower than 100,000 W/cm² and, more preferably, not lower than 200,000 W/cm², each on the focal plane. An exposure speed is, preferably, not slower than 1 ms⁻¹. and, more preferably, not slower than 2 ms⁻¹.

A preferable example of the exposure conditions may be given as follows. However, the exposure conditions shall not be limited thereto.

| Output power (mW) | Optical efficiency (%) | Exposure spot diameter (µm) | Power density on focal plane (W/cm²) |
|---|---|---|---|
| 100 | 50 | 6 | 177000 |
| 150 | 70 | 10 | 134000 |
| 500 | 50 | 10 | 318000 |
| 2000 | 30 | 10 | 764000 |

An ablation produced by making a high intensity exposure may be in the halftone dot form or may also be in the continuously ablation form.

When applying heat to the whole surface of a recording material and an image-receiving material each put one upon another, the heat energy may be applied from any side of the image-receiving material, recording material or both of the materials. By applying the above-mentioned heat, the thermally diffusible dye of a colorant layer is diffused to be transferred to the image-receiving layer of the image-receiving material from a colorant layer through the foregoing ablation of a colorant barrier layer, so that an image can be formed. There is no special limitation to a heating temperature. However, it is to be within the range of, ordinarily, 60 to 200°C and, preferably, 80 to 150°C.

### EXAMPLES

In the following descriptions, the term, "a part" or "parts", herein means "a part by weight" or "parts by weight".

### Example 1

### Preparation of a recording element

The following compositions were mixed up and dispersed together, so that a colorant layer coating solution containing a thermally diffusible dye could be prepared.

### Colorant layer coating solution

| | |
|---|---|
| Thermally diffusible dye (Kayaset-blue 714 manufactured by Nihon Kayaku Co.) | 4 parts |
| Polyvinyl butyral resin (Eslec BX-1 manufactured by Sekisui Chemical Co.) | 4 parts |
| Methyl ethyl ketone | 90 parts |
| Cyclohexanone | 10 parts |

The above-mentioned colorant layer coating solution was coated on a 100µm-thick polyethylene terephthalate (PET) film by making use of a wire-bar and then dried up, so that a 4µm-thick colorant layer was formed. On the rear side of the PET film, there was formed a nitrocellulose layer containing a silicone-denatured urethane resin (SP-2105 manufactured by Dai-Nichi Seika Co.).

Next, a recording element was prepared in the following manner. A colorant barrier layer having the following composition was coated on the above-mentioned colorant layer by making use of a wire-bar and then dried up, so that a 0.5µm-thick colorant barrier layer was formed.

### Colorant layer coating solution

### Preparation of an image-receiving element

An image-receiving material was prepared in the following manner. On a 150µm-thick synthetic paper (Upo FPG-150 manufactured by Oji Yuka Synthetic Paper Co.), a coating solution for forming an image-receiving layer, which has the following composition, was coated by making use of a wire-bar. The resulting coated synthetic paper was preliminarily dried by making use of a drier, and was then dried up in an oven at 100°C for one hour, so that a 5µm-thick image-receiving layer was formed on the synthetic paper.

### Coating solution for forming an image-receiving layer

| | |
|---|---|
| Vinyl chloride-vinyl isobutylether copolymer (Laroflex MP25 manufactured by BASF) | 9 parts |
| A polyester-denatured silicone resin (X-24-8300 manufactured by Shinetsu Silicone Co.) | 1 part |
| Methyl ethyl ketone | 40 parts |
| Cyclohexanone | 10 parts |

### (Formation of an image)

### 〈Ablation of the colorant barrier layer〉

The colorant barrier layer was ablated in the following manner. A laser beam of a semiconductive laser LT090MD/MF, having a wavelength of 830nm and the maximum beam output of 100mW, manufactured by Sharp Corp., was so condensed as to be a beam having an approximately 6µm-diameter. The resulting laser beam was applied at a scanning speed of 2ms⁻¹. to the colorant barrier layer of the resulting recording material. At that time, the optical efficiency was 60%. The dot size in the portions where the ablation was made dotwise was 8µm.

### 〈Transfer of the colorant〉

As mentioned above, the recording element of which the colorant barrier layer was ablated and the image-receiving material were put one upon another so that the colorant barrier layer and the image-receiving layer could be brought into contact with each other. Then, only the colorant, that was the diffusible dye, in the ablated portion were transferred to the image-receiving layer through a heat roll capable of applying heat of 120°C and pressure of 2 kg/cm².

When measuring the red reflection density in the over-all solid transferred portion, or the over-all solid density, it was proved to be 2.3. When measuring the reflection density in the unablated portion or the white background density, it was proved to be 0.06. The above-mentioned reflection density was also proved to remain unchanged from the reflection density of the image-receiving element measured before it was passed through the heat roll.

### Example 2

The preparation steps from the beginning to the preparation of the colorant layer were quite the same as in Example 1. However, three kinds of the recording elements of the invention and one kind of the comparative recording element were prepared by changing only the composition of the colorant barrier layers as given below. The colorant barrier layers were each made to have a thickness of 0.5µm.

### Recording element 2-1

| | |
|---|---|
| Polycarbonate resin (w/Tg 140°V) (IUPILON S2000 manufactured by Mitsubishi Gas-Chemical Co.) | 4 parts |
| Near-infrared absorbable dye (IR-2) | 1 part |
| Methylene chloride | 95 parts |

### Recording element 2-2

| | |
|---|---|
| Water-soluble polyester resin (w/anionic property and pH=3 to 5), (Pesresin 200 in an aqueous 20% solution, manufactured by Takamatsu Yushi Co.) | 20 parts |
| Infrared absorbable dye (IR-3) | 1 part |
| Pure water | 79 parts |

### Recording material 2-3

| | |
|---|---|
| Methyl cellulose resin (SM400 manufactured by Shinetsu Chemical Co.) | 3 parts |
| Infrared absorbable dye (IR-4) | 2 parts |
| Pure water | 95 parts |

### Recording element for comparison

By making use of the above-mentioned recording elements and the same image-receiving material as in Example 1, the ablation of the colorant layers and the thermal transfer to the image-receiving layers each quite the same as in Example 1 were carried out, respectively. The results thereof will be given below.

| Recording element | Solid density | White background density | Spot size in the ablated portion (µm) |
|---|---|---|---|
| 2-1 | 2.4 | 0.06 | 4.5 |
| 2-2 | 2.5 | 0.07 | 6.0 |
| 2-3 | 2.3 | 0.06 | 6.0 |
| Comparison | - | 2.0 | 0 |

In the comparative recording element, any infrared absorbable substance was not contained. Therefore, no ablation could be found out. In the colorant barrier layer, there was no barrier effect. Therefore, the dye having a considerable density was transferred to the image-receiving layer.

### Example 3

### Preparation of a recording element

A recording element the same as that in Example 1 was prepared.

An image-receiving element was prepared in the following manner. On a 150µm-thick synthetic paper (Upo FPG-150 manufactured by Oji Yuka Synthetic Paper Co.), a coating solution for forming an image-receiving layer, which has the following composition, was coated by making use of a wire-bar. The resulting coated synthetic paper was preliminarily dried by making use of a drier, and was then dried up in an oven at 100°C for one hour, so that a 5µm-thick image-receiving layer was formed on the synthetic paper.

### Coating solution for an image-receiving layer

| | |
|---|---|
| Vinyl chloride-vinyl isobutylether copolymer (Laroflex MP25 manufactured by BASF) | 8.5 parts |
| Globular-shaped fine particles of polymethyl methacrylate (w/particle size of 12-15µm) | 0.5 parts |
| Polyester-denatured silicone resin (X-24-8300 manufactured by Shinetsu Silicone Co.) | 1 part |
| Methyl ethyl ketone | 40 parts |
| Cyclohexanone | 10 parts |

The resulting recording element and the image-receiving element were contacted at the colorant barrier surface and image receiving layer surface and unified into a body at 90°C through a heat roll with a pressure of 1 kg/cm².

### (Formation of an image)

### 〈Ablation of the colorant barrier layer〉

The colorant barrier layer was ablated in the following manner. A laser beam of a semiconductive laser LT090MD/MF (having a wavelength of 830nm and the maximum beam output of 100mW, manufactured by Sharp Corp.) was so condensed to the colorant barrier layer as to be a beam having an approximately 6µm-diameter at the time of the maximum output. The resulting laser beam was applied, at a scanning pitch of 10µm and a scanning speed of 2m/second, to the colorant barrier layer of the resulting recording element. (At that time, the optical efficiency was 60%).

### 〈Transfer of a colorant〉

The elements unified into a body, of which the colorant barrier layer was ablated, was passed through a heat roll capable of applying heat of 130°C and a pressure of 3 kg/cm², so that only the colorants in the ablated portions, which were diffusible dyes, were transferred to the image-receiving layer.

The unified two elements were peeled off
When measuring the red reflection density in the transferred solid image portion comprised of 8µm-sized dots or the solid density, it was proved to be 3.1. When measuring the reflection density in the unablated portion (or the white background density), it was proved to be 0.06, that was also proved to remain unchanged from the reflection density of the image-receiving material measured before it was passed through the heat roll.

### Example 4

### Preparation of a recording element

A colorant layer coating solution containing a thermally diffusible dye was prepared by mixing and dispersing the following compositions.

### Colorant layer coating solution

| | |
|---|---|
| Thermally diffusible dye (D-1) | 25 parts |
| Ditto (D-2) | 15 parts |
| Ditto (D-3) | 40 parts |
| Polyvinyl butyral resin (Eslec BX-1) | 20 parts |
| Methyl ethyl ketone | 700 parts |
| Cyclohexanone | 200 parts |

The above-mentioned colorant layer coating solution was coated on a 100µm-thick PET film by making use of a wire-bar and then dried up, so that a 4µm-thick colorant layer could be prepared.

Next, a recording material was prepared in the following manner. A colorant barrier layer coating solution having the following composition was coated on the above-mentioned colorant layer by making use of a wire-bar and then dried up, so that a 0.15µm-thick colorant barrier layer could be so prepared as to complete the recording element.

### Colorant barrier layer coating solution

| | |
|---|---|
| Gelatin | 2.5 parts |
| Infrared absorbable dye (IR-3) | 2.0 parts |
| Colloidal silver | 0.5 parts |
| Pure water | 95 parts |

### Preparation of an image-receiving element

A 100µm-thick PET film of which the rear surface was treated in an antistaticity prevention process, and the surface resistance thereof was set to be 10¹⁰Ω. An image-receiving layer coating solution having the following composition was coated, by making use of a wire-bar, on the surface of the PET film opposite to the antistaticity prevented surface thereof, and then dried up at 120°C for 30 minutes, so that a 4µm-thick image-receiving layer was formed.

### Image-receiving layer coating solution

| | |
|---|---|
| Polyvinyl butyral (Eslec BL-1 manufactured by Sekisui Chemical Co.) | 40 parts |
| Metal source (D-4) | 50 parts |
| Amino-modified silicone (KF-393 manufactured by Shinetsu Silicone Co.) | 5 parts |
| Epoxy-modified silicone (X-22-343 manufactured by Shinetsu Silicone Co.) | 5 parts |
| Methyl ethyl ketone | 300 parts |
| Cyclohexanone | 100 parts |

### Formation of an image

### 〈Ablation of the colorant barrier layer〉

The colorant barrier layer of the above-mentioned recording material was exposed to light when a semiconductive laser beam having a wavelength of 810nm and the maximum beam output of 150mW was condensed so that a beam diameter of the half-band width could be 5µm at the time of the maximum output having an approximately 6µm-diameter. The exposure was made by 16 semiconductive laser beams.

When making the exposure, the light output on the focal plane was proved to be 101 mW in average per semiconductive laser. The exposure energy density, obtained by calculating out from the exposure light scanning speed, was proved to be 150 mJ/cm², when making an over-all solid exposure.

### 〈Transfer of a colorant〉

As mentioned above, the colorant barrier layer of a recording material, of which the colorant barrier layer was ablated, and the image-receiving layer of an image-receiving material were put one upon another so that the layers could be brought into contact with each other. Then, only the colorants in the ablated portion were transferred to the image-receiving layer through a heat roll capable of applying heat of 180°C and pressure of 2 kg/cm².

The transmission densities were proved to be 0.02 of the PET film, 0.04 in the unexposed portions, and 3.28 in the over-all solid exposed portions, respectively. Further for the purpose of confirming the preservability of the resulting images, the images were preserved at 50°C for one month. Resultingly, the preservability was excellently displayed without any image bleeding, even as compared to the reference to a preservation at room temperature.

### Example 5

A recording material was prepared on a 12µm-thick PET film in the same manner as in Example 4, except that only the composition of the colorant layer coating solution was changed as follows. Also, the following image-receiving element was prepared.

### Colorant layer coating solution

| | |
|---|---|
| Thermally diffusible dye (D-1) | 22 parts |
| Ditto (D-2) | 13 parts |
| Ditto (D-3) | 35 parts |
| Matting agent (MR-20G having an average particle size of 17µm, manufactured by Soken Chemical Co.) | 10 parts |
| Polyvinyl butyral resin (Eslec BX-1) | 20 parts |
| Methyl ethyl ketone | 700 parts |
| Cyclohexanone | 200 parts |

### (Preparation of an image-receiving element)

A 175µm-thick PET film, of which the rear surface was treated in an antistaticity prevention process and the surface resistance thereof was set to be 5x10⁹Ω. A cushion layer coating solution having the following composition was coated, by making use of a doctor-blade, on the surface of the PET film opposite to the staticity prevented surface thereof, so that a 10µm-dried-thick cushion layer was formed.

### Cushion layer coating solution

| | |
|---|---|
| Ethylene-vinyl acetate resin (Evaflex EV-40Y manufactured by Mitsui-DuPont Polychemical Co.) | 30 parts |
| Toluene | 60 parts |
| Methyl ethyl ketone | 10 parts |

Next, apart from the above, a 25µm-thick PET film was provided with a peelability by applying a silicone surface treating agent. On the surface treating agent coated surface thereof, an image-receiving layer coating solution having the following composition was coated by making use of a wire-bar, so that a 3µm-dried-thick image-receiving layer was formed.

### Image-receiving layer coating solution

| | |
|---|---|
| Vinyl chloride resin (TK-300 manufactured by Shinetsu Chemical Co.) | 40 parts |
| Metal source (D-4) | 50 parts |
| Amino-modified silicone (KF-393 manufactured by Shinetsu Silicone Co.) | 5 parts |
| Epoxy-modified silicone (X-22-343 manufactured by Shinetsu Silicone Co.) | 5 parts |
| Methyl ethyl ketone | 300 parts |
| Cyclohexanone | 100 parts |

The surface of the image-receiving layer provided onto the 25µm-thick peelable PET film and the surface of the previously formed cushion layer of the 175µm-thick PET film were each made face to face and were then applied with a pressure of 3 kg/cm² by a laminator at room temperature, so that the two sheets thereof were pasted together. Thereafter, the peelable PET film was peeled off, so that an image-receiving element comprising a cusion layer and an image-receiving layer each formed in this order on a 175µm-thick PET film could be prepared.

### Unification process

Now, the surface of the barrier layer of the recording element and the surface of the image-receiving layer of the image-receiving element were made face to face and they were then applied with a pressure of 0.5 kg/cm² by making use of a laminator at room temperature, so that the recording material and the image-receiving element were unified into a body.

### Formation of an image

The colorant barrier layer was ablated in the same manner as in Example 4, and the unified material was applied with a heat of 180°C and a pressure of 5 kg through a laminator. Thereafter, the both of the materials were separated from each other. The transmission densities were proved to be 0.02 of the PET film, 0.04 in the unexposed portions, and 3.14 in the over-all solid exposed portions, respectively.

### Comparative Example 1

A colorant layer coating solution for a recording element, to which a colorant layer whole can be exploded to be transferred, was prepared by mixing and dispersing the following compositions. The resulting coating solution was coated in an aluminium-evaporated layer which was evaporated on a 100µm-thick polyester film so as to have a transmission density of 50%.

### Colorant layer coating solution

| | |
|---|---|
| Carbon black | 7 parts |
| Phenol resin (Tamanol 510 manufactured by Arakawa Chemical Co.) | 3 parts |
| Methyl ethyl ketone | 40 parts |

As for the image-receiving material, an unprocessed polyester film was used as it was.

### Image recording

The foregoing recording material and the image receiving material were put on upon another, and then the air remaining in the interspace between the two sheets of the material was evacuated by making close contact under reduced pressure so as to bring them into close contact with each other. From the rear side of the recording material, an aluminium-evaporated layer was exposed to a semiconductive laser beam condensed (to have a wavelength of 810µm and the maximum beam output of 150mW) so that the beam diameter of the half-band width could be 5µm at the time of the maximum output. When making an exposure, 16x16 dots (that is, 256 dots in total) each having a spot diameter of 5µm were taken as a pixel unit, and an image was formed in terms of 80µm square units. At that time, the exposure surface power was proved to be 101mW. The over-all solid densities in the over-all solid portions were obtained as relatively high as could be 2.85. However, there were may pin-holes, so that image uniformity was not satisfactory.

## Claims

1. A thermal transfer image recording method comprising the steps of
imagewise exposing a recording element to high intensity light, which comprises a support (1) having thereon a colorant layer (2) containing a colorant, and a colorant barrier layer (3) comprising an infrared absorbing substance and a resin in an amount of 50 % to 99 % by weight of the total weight of the colorant barrier layer (3) and being provided on said colorant layer (2), to imagewise ablate said colorant barrier layer (3)
contacting the surface of said colorant barrier layer (3) with the surface of the image receiving layer (5) of an image receiving element (4), and
transferring the colorant of said colorant layer (2) through the ablated portion of said colorant barrier layer (3) to said image receiving layer (5) by applying heat or pressure.

2. The method of claim 1, wherein said colorant barrier layer (3) comprises a water-soluble resin.

3. The method of claim 2, wherein said water-soluble resin is selected from the group consisting of gelatin, polyvinyl alcohol, water-soluble polyvinyl formal, water-soluble polyvinyl-acetal, water-soluble polyvinylbutyral, polyvinyl-pyrrolidone, water-soluble polyester, water-soluble nylon, polyacrylic acid, water-soluble polyurethane, methylcellulose, hydroxyethylcellulose, hydroxypropylcellulose and carboxylcellulose.

4. The method of claim 1, wherein said colorant barrier layer (3) comprises a resin having an acidic group selected from -COO⁻, -SO₃⁻ and -PO₃⁻, or a basic group selected from -NH₂, -NH- and -N=.

5. The method of claim 1, wherein said colorant barrier layer (3) comprises a resin having a glass transition point of not lower than 120°C.

6. The method of claim 1, wherein said colorant layer (2) comprises a dye capable of forming a chelate compound.

7. The method of claim 1, wherein said infrared absorbing substance is a dye having an absorption maximum within the range of from 700 nm to 1200 nm and a molar extinction coefficient of 50,000 or more at the maximum absorption wavelength.

8. The method of claim 1, wherein said image receiving layer (5) contains a metal ion-containing compound

9. The method of claim 1, wherein said exposing step is carried out by high intensity light having a power density of not less than 100 000 W/cm² with an exposing speed of not less than 1 ms⁻¹.

## Patentansprüche

1. Bildaufzeichnungsverfahren durch Thermotransfer, umfassend folgende Stufen:
Bildgerechtes Belichten eines Aufzeichnungsmaterials aus einem schichtträger (1) mit einer darauf befindlichen und ein Färbemittel enthaltenden Färbemittelschicht (2) und einer auf der Färbemittelschicht (2) vorgesehenen, eine infrarotabsorbierende Substanz und ein Harz in einer Menge von 50 bis 99 Gew.-% ihres Gesamtgewichts enthaltenden Färbemittelsperrschicht (3) mit Licht hoher Intensität zur bildgerechten Abtragung der Färbemittelsperrschicht (3);
Kontaktieren der Oberfläche der Färbemittelsperrschicht (3) mit der Oberfläche einer Bildempfangsschicht (5) eines Bildempfangsmaterials (4) und
Übertragen des Färbemittels der Färbemittelschicht (2) durch den abgetragenen Teil der Färbemittelsperrschicht (3) hindurch auf die Bildempfangsschicht (5) durch Applikation von Wärme oder Druck.

2. Verfahren nach Anspruch 1, wobei die Färbemittelsperrschicht (3) ein wasserlösliches Harz enthält.

3. Verfahren nach Anspruch 2, wobei das wasserlösliche Harz aus der Gruppe Gelatine, Polyvinylalkohol, wasserlösliches Polyvinylformal, wasserlösliches Polyvinylacetal, wasserlösliches Polyvinylbutyral, Polyvinylpyrrolidon, wasserlöslicher Polyester, wasserlösliches Nylon, Polyacrylsäure, wasserlösliches Polyurethan, Methylcellulose, Hydroxyethylcellulose, Hydroxypropylcellulose und Carboxylcellulose ausgewählt ist.

4. Verfahren nach Anspruch 1, wobei die Färbemittelsperrschicht (3) ein Harz mit einer sauren Gruppe, ausgewählt aus -COO⁻, -SO₃⁻ und -PO₃⁻, oder einer basischen Gruppe, ausgewählt aus -NH₂, -NH- und -N=, enthält.

5. Verfahren nach Anspruch 1, wobei die Färbemittelsperrschicht (3) ein Harz einer Einfriertemperatur von nicht unter 120°C enthält.

6. Verfahren nach Anspruch 1, wobei die Färbemittelschicht (2) einen zur Bildung einer Chelatverbindung fähigen Farbstoff enthält.

7. Verfahren nach Anspruch 1, wobei die infrarotabsorbierende Substanz aus einem Farbstoff eines Absorptionsmaximums innerhalb des Bereichs von 700 nm bis 1200 nm und eines molaren Extinktionskoeffizienten von 50000 oder mehr bei der Absorptionsmaximumwellenlänge besteht.

8. Verfahren nach Anspruch 1, wobei die Bildempfangsschicht (5) eine metallionenhaltige Verbindung enthält.

9. Verfahren nach Anspruch 1, wobei die Belichtung mit Licht hoher Intensität einer Leistungsdichte von nicht weniger als 100000 W/cm² bei einer Belichtungsgeschwindigkeit von nicht weniger als 1 ms⁻¹ durchgeführt wird.

## Revendications

1. Procédé d'enregistrement d'une image par transfert thermique comprenant les étapes consistant à :
exposer un élément d'enregistrement à une lumière à haute intensité, sous la forme d'une image, cet élément d'enregistrement comprenant un support (1) ayant une couche (2) de colorant contenant un colorant, et une couche (3) constituant une barrière au colorant contenant une substance absorbant les infrarouges et une résine, représentant de 50% à 99% en poids du poids total de la couche (3) constituant une barrière au colorant et disposée sur ladite couche (2) de colorant, pour enlever suivant l'image ladite couche (3) constituant une barrière au colorant,
mettre en contact la surface de ladite couche (3) constituant une barrière au colorant avec la surface de la couche (5) pour recevoir l'image, d'un élément (4) pour recevoir une image et
transférer le colorant de ladite couche (2) de colorant à travers la portion enlevée de ladite couche (3) constituant une barrière au colorant à ladite couche (5) pour recevoir l'image, par application de chaleur ou de pression.

2. Procédé de la revendication 1, où ladite couche (3) constituant une barrière au colorant contient une résine hydrosoluble.

3. Procédé de la revendication 2, où ladite résine hydrosoluble est choisie dans le groupe constitué par une gélatine, un alcool polyvinylique, un formal polyvinylique hydrosoluble, un acétal polyvinylique hydrosoluble, un butyral polyvinylique hydrosoluble, une polyvinylpyrrolidone, un polyester hydrosoluble, un nylon hydrosoluble, un acide polyacrylique, un polyuréthanne hydrosoluble, une méthylcellulose, une hydroxyéthylcellulose, une hydroxypropylcellulose et une carboxycellulose.

4. Procédé de la revendication 1, où ladite couche (3) constituant une barrière au colorant contient une résine ayant un groupe acide choisi parmi -COO⁻, -SO₃⁻ et PO₃⁻, ou un groupe basique choisi parmi -NH₂, -NH- et -N=.

5. Procédé de la revendication 1, où ladite couche (3) constituant une barrière au colorant contient une résine ayant une température de transition vitreuse qui n'est pas inférieure à 120°C.

6. Procédé de la revendication 1, où ladite couche (2) de colorant contient un colorant capable de former un chélate.

7. Procédé de la revendication 1, où ladite substance absorbant les infrarouges est un colorant ayant un maximum d'absorption dans la plage allant de 700 nm à 1200 nm et un coefficient d'extinction molaire de 50.000 ou plus à la longueur d'absorption maximum.

8. Procédé de la revendication 1, où ladite couche (5) pour recevoir l'image contient un composé contenant un ion métallique.

9. Procédé de la revendication 1, où ladite étape d'exposition se fait avec une lumière à haute intensité, ayant une densité de puissance qui n'est pas inférieure à 100.000 W/cm², avec une vitesse d'exposition qui n'est pas inférieure à 1 ms⁻¹.
